

July 19, 1949.

C. KELLER  
TUBING FOR HEAT EXCHANGERS OPERATED  
AT HIGH TEMPERATURES AND PRESSURES  
Filed Jan. 14, 1946

2,476,666

Fig. 1



Fig. 3



Fig. 2



Fig. 4

Inventor  
Curt Keller

23

Dodge Cur. Inc.

Attorneys

## UNITED STATES PATENT OFFICE

2,476,666

## TUBING FOR HEAT EXCHANGERS OPERATED AT HIGH TEMPERATURES AND PRESSURES

Curt Keller, Kusnacht, Switzerland, assignor to Aktiengesellschaft Fuer Technische Studien, Zurich, Switzerland, a corporation of Switzerland

Application January 14, 1946, Serial No. 641,108

3 Claims. (Cl. 138—38)

1

This invention relates to heat transfer tubes for use under conditions in which the exterior of the tube must have good resistance to corrosion by hot flue gases and slag and the tube must have good creep resistance at high temperatures.

The tube is intended for use in heaters forming a part of closed circuit power plants of the type described in applicant's Patent No. 2,172,910, issued on September 12, 1939.

The working medium is usually air which passes through the heater under pressures ranging from 600 to 1000 p. s. i. and leaves the heater at temperatures as high as 1300° F. Thus the tube temperatures are well over 1000° F. and as ordinarily designed the metal of the tubes is stressed in tension from 2500 to 5000 pounds per square inch.

To secure adequate creep resistance recourse has been had to high alloy steels; for example, steels containing 18% chrome and 8% nickel or even higher percentages of alloying metal have been used.

Alloys of this type are corroded by sulfur compounds in the products of combustion of coals and many oils and also are attacked actively by slags and ash particles.

There are, however, plain chrome alloy steels which resist such corrosion. A satisfactory chrome content is 20-30%. The expense of welding a surface layer of chrome alloy steel to a chrome-nickel alloy steel core is heavy and indeed almost prohibitive. The present invention is based on the discovery that this is not necessary. A separate envelope can be made to give excellent heat transfer and has an added advantage in that it can be replaced. The concept stems from observation of the fact that suitable chrome alloy steels have coefficients of thermal expansion only about half those of suitable chrome-nickel steels.

The basic concept is a tubular core of creep-resistant steel with a thin envelope of corrosion-resistant steel closely encircling the core at ordinary temperatures and having a lower thermal coefficient of expansion, so that at the high working temperature the envelope is stressed into close contact with the core, assuring good heat transfer.

As a further detail the envelope is wrapped on the core, either in the form of a longitudinal strip whose edges are seamed or locked together, or in the form of a strip helically wound with a slight lap at the edges. The described procedures are preferred because it is difficult to telescope together a preformed tubular core and

2

preformed tubular envelope and secure the desired close fit. Even if this can be done on a commercial basis, the life of the envelope is the life of the tube.

5 To afford a better understanding of the invention, typical constructions will be described by reference to the accompanying drawing in which:

Fig. 1 is an elevation of a tube having a longitudinally seamed envelope.

10 Fig. 2 is a transverse section thereof.

Fig. 3 is an elevation of a tube having a helically wound envelope.

15 Fig. 4 is a transverse section of the tube shown in Fig. 3.

20 In all the figures the part 6 is a tubular core of creep resisting alloy steel, for example chrome-nickel alloy steel of the composition suggested above and of a thickness appropriate to the internal pressure to be encountered and to the tube diameter.

In Figs. 1 and 2 the envelope 7 is of corrosion resisting chrome alloy steel, stretched in tension around the core and longitudinally seamed at 8. The strip is approximately 0.01 inch in thickness.

25 An ordinary lock seam is indicated, but details of the seam may be varied.

In Figs. 3 and 4 the envelope 9 is a strip of chrome alloy steel of similar thickness wound helically under tension, successive convolutions overlapping slightly as shown at 11. To prevent unwinding it is desirable to tack weld the helically wound strip at intervals as indicated at 12. The intervals are such as to allow the strip to accommodate itself to minor flexures of the core.

35 If either type of envelope burns out, it can be stripped from the core and a new envelope can be applied without dismantling the heater.

In any heater in which tubes are expanded in headers or welded therein, the possibility of applying the envelope to cores after the cores are fixed in the headers is a very useful feature of the invention.

What is claimed is:

1. A heat transfer tube for use in heaters for gases under pressure in which the wall temperature of the tube is 1000° F. or higher and the stress on the metal of the tube is from 2500 to 5000 pounds per square inch; said tube comprising a stress resisting core of alloy steel characterized by good creep resistance; and a thin envelope free of said core and composed of an alloy steel having good resistance to the corrosive effects of slag and combustion gases, said envelope being in close contact with said core at atmospheric temperatures and having a coefficient of

thermal expansion materially lower than that of the core, whereby the envelope is stressed at the operating temperatures and good heat transfer is assured.

2. A tube as defined in claim 1 in which the envelope is a strip tightly wrapped upon the core when cold and having a longitudinal locked seam.

3. A tube as defined in claim 1 in which the envelope is a strip wound helically on the core, and under tension when cold, the edges of said strip having an overlap.

## REFERENCES CITED

The following references are of record in the file of this patent:

## UNITED STATES PATENTS

| Number    | Name       | Date          |
|-----------|------------|---------------|
| 432,059   | Maschmeyer | July 15, 1890 |
| 1,839,964 | Harvey     | Jan. 5, 1932  |
| 2,139,538 | Becket     | Dec. 6, 1936  |
| 2,258,564 | Armstrong  | Oct. 7, 1941  |

CURT KELLER.